

# United States Patent

von König et al.

[15] 3,647,451

[45] Mar. 7, 1972

[54] **ANTIBRONZING AGENTS FOR  
PHOTOGRAPHIC SILVER IMAGES**

[72] Inventors: Anita von König, Leverkusen; **Helmut Timmler**, Wuppertal-Vohwinkel, both of Germany

[73] Assignee: **Agfa-Gevaert Aktiengesellschaft**, Leverkusen, Germany

[22] Filed: **Mar. 21, 1969**

[21] Appl. No.: **809,415**

[30] **Foreign Application Priority Data**

Mar. 28, 1968 Germany ..... P 17 70 074.2

[52] U.S. Cl. .... **96/52, 96/61, 96/66,  
96/67**

[51] Int. Cl. .... **G03c 7/00, G03c 5/38, G03c 1/76**

[58] **Field of Search** ..... **96/52, 67, 61, 66**

[56] **References Cited**

UNITED STATES PATENTS

2,514,650 7/1950 Knott ..... **96/52**  
3,438,777 4/1969 Willems ..... **96/52**

*Primary Examiner*—Norman G. Torchin

*Assistant Examiner*—Mary F. Kelley

*Attorney*—Connolly and Hutz

[57] **ABSTRACT**

Antibronzing agents for silver images dried at high temperatures, which agents have 1,3,4-triazole-3-mercaptan rings bridged together at their 5-positions by an interrupted hydrocarbon linkage.

**8 Claims, No Drawings**

## ANTIBRONZING AGENTS FOR PHOTOGRAPHIC SILVER IMAGES

The invention relates to a process for the production of photographic images which includes drying on a high-gloss press at high temperature in effective contact with antibronzing agents of the bis-mercapto triazole series.

The silver images obtained from light-sensitive silver halide emulsion layers often undergo changes during high-gloss drying or during mechanical drying at high temperature. Thus commonly a loss in density occurs or blue-black image tones change to brownish tones and brown tones change into greenish black tones. These changes are known as "partial burning" or "bronzing" of the silver image.

The incorporation of small quantities of certain chemical compounds, known as antibronzing agents, into the light-sensitive material which contains a silver halide emulsion copying layer is known. These compounds alternatively may be added to the treatment baths which are used for the material to prevent this loss of density.

The known antibronzing compounds are however, only of limited utility either because their antibronzing effect is not sufficient or because they impair the photographic properties.

It is among the objects of the present invention to provide new antibronzing agents which have a sufficiently large antibronzing effect and which do not deleteriously effect the photographic properties of the material.

We now have found that heteroalkylene-5,5'-bis-1,2,4-triazole-3-mercaptans of the following formula are outstanding antibronzing agents.



in which

R represents (1) hydrogen, (2) a saturated or olefinically unsaturated aliphatic group having 1-18 carbon atoms and preferably one to six carbon atoms, (3) aryl such as a phenyl or naphthyl particularly a radical of the phenyl series, (4) aralkyl such as a benzyl or phenylethyl group, (5) cycloalkyl, such as a cyclohexyl group or (6) an amino group; these hydrocarbon radicals may also be substituted, e.g., with halogen, methyl, methoxy, hydroxyl, sulfo or carboxy groups;

X stands for a hydrocarbon chain such as alkylene, arylene, for example phenylene, or cycloalkylene. Preferred are aliphatic chains having 2-10 methylene groups in particular aliphatic chains which are interrupted by one or more preferably one to three heteroatoms such as oxygen, sulfur or imino or sulfonyl groups.

The above formula includes compounds in the tautomeric 3-thione form.

Examples of suitable compounds are shown in the following table:

The preparation of heteroalkylene-5,5'-bis-1,2,4-triazole-3-mercaptans, is carried out in a manner analogous to the preparation of 5-substituted 1,2,4-triazole-3-mercaptans. The corresponding carboxylic acid esters which are used as starting materials, are cyclized with thiosemicarbazides or thiocarbohydrazide (Pesson, Dupin and Polmans, Bull. Soc. Chim. France (5) 1581 (1961)).

The preparation of Compound 14 is described in the following in detail:

10 Ninety-one grams of thiosemicarbazide and 89 g. of dimethylthiodiglycolate are added to a solution of 23 g. of sodium dissolved in 2 liters of ethanol. The reaction mixture is refluxed for 12 hours. After cooling, it is suction-filtered and the filtrate is concentrated by evaporation. The combined residues are dissolved in water and the reaction product is precipitated by the introduction of carbonic acid. Sixty grams of bis[3-mercapto-1,2,4-triazolyl-(5)-methyl]-sulfide are obtained.

15 The other compounds given in the table are obtained by similar processes.

20 The antibronzing agents are preferably added to the light-sensitive silver halide emulsion layer. They may be added to the emulsion, preferably after the chemical ripening, or to the finished casting solution. The compounds are preferably used in solution in a suitable solvent such as water, alcohol, dimethylformamide or in an equivalent quantity of aqueous alkali.

25 The amount of the antibronzing agent is not critical and depends on the type of the silver halide emulsion or the effects desired. In general quantities of 1/50th to 1/1,000th of a mol per mol of silver halide, preferably 1/100 to 1/500th mol per mol of silver halide, that is 0.1-5 g., preferably 0.5-2.5 g. per mol of silver halide have proved sufficient.

30 The compounds may also be added to auxiliary water-permeable layers of the photographic material, e.g., to the baryta coating or to a protective layer. The antibronzing agents of the invention may be added to any of the conventional silver halide emulsions. Examples of suitable silver halides are silver chloride, silver bromide or mixtures of the halides which may contain a certain amount of silver iodide, preferably up to about 10 mols percent.

35 The binding agent for the light-sensitive silver halide emulsion layer is preferably gelatin but this may be partly replaced by other film-forming natural or synthetic polymers. Suitable agents for this purpose are, e.g., alginic acid and its derivatives such as its salts, esters or amides, carboxymethyl cellulose, alkyl cellulose, starch and starch derivatives, polyvinyl alcohol, copolymers with vinyl alcohol and vinyl acetate units, polyvinyl pyrrolidone and the like.

40 The silver halide emulsion may contain any known additives, such as antifogging agents, stabilizers, hardeners, plasticizers and wetting agents. The emulsion may also be both chemically and spectrally sensitized. It can be chemically sensitized by carrying out the ripening in the presence of small quantities of sulfur containing compounds, such as allyl isothiocyanate, allylthioether or sodium thiosulfate. The light-sensitive silver halide emulsion may also be sensitized with

TABLE 1

| Compound Number | R                                     | X                                                                       | M.P. or decomposition point, degrees |
|-----------------|---------------------------------------|-------------------------------------------------------------------------|--------------------------------------|
| 1.....          | CH <sub>3</sub>                       | -CH <sub>2</sub> -S-CH <sub>2</sub> -                                   | 265                                  |
| 2.....          | CH <sub>2</sub> =CH-CH <sub>2</sub> - | -CH <sub>2</sub> -S-CH <sub>2</sub> -                                   | 178                                  |
| 3.....          | C <sub>6</sub> H <sub>5</sub>         | -CH <sub>2</sub> -S-CH <sub>2</sub> -                                   | 282                                  |
| 4.....          | NH <sub>2</sub>                       | -CH <sub>2</sub> -S-CH <sub>2</sub> -                                   | 251                                  |
| 5.....          | H-                                    | -CH <sub>2</sub> -CH <sub>2</sub> -S-CH <sub>2</sub> -CH <sub>2</sub> - | 281                                  |
| 6.....          | CH <sub>3</sub>                       | -CH <sub>2</sub> -CH <sub>2</sub> -S-CH <sub>2</sub> -CH <sub>2</sub> - | 225                                  |
| 7.....          | C <sub>6</sub> H <sub>5</sub>         | -CH <sub>2</sub> -CH <sub>2</sub> -S-CH <sub>2</sub> -CH <sub>2</sub> - | 263                                  |
| 8.....          | CH <sub>2</sub> =CH-CH <sub>2</sub> - | -CH <sub>2</sub> -CH <sub>2</sub> -S-CH <sub>2</sub> -CH <sub>2</sub> - | 192                                  |
| 9.....          | NH <sub>2</sub>                       | -CH <sub>2</sub> -CH <sub>2</sub> -S-CH <sub>2</sub> -CH <sub>2</sub> - | 225                                  |
| 10.....         | NH <sub>2</sub>                       | -CH <sub>2</sub> -O-CH <sub>2</sub> -                                   | 219                                  |
| 11.....         | CH <sub>3</sub>                       | -CH <sub>2</sub> -S O <sub>2</sub> -CH <sub>2</sub> -                   | 235                                  |
| 12.....         | H-                                    | -CH <sub>2</sub> -S-CH <sub>2</sub> -S-CH <sub>2</sub> -                | 271                                  |
| 13.....         | NH <sub>2</sub>                       | -CH <sub>2</sub> -S-CH <sub>2</sub> -S-CH <sub>2</sub> -                | 203                                  |
| 14.....         | H                                     | -CH <sub>2</sub> -S-CH <sub>2</sub> -                                   | 317                                  |
| 15.....         | C <sub>6</sub> H <sub>5</sub>         | -CH <sub>2</sub> -S-CH <sub>2</sub> -S-CH <sub>2</sub> -                | 268                                  |
| 16.....         | CH <sub>2</sub> =CH-CH <sub>2</sub> - | -CH <sub>2</sub> -S-CH <sub>2</sub> -S-CH <sub>2</sub> -                | 141                                  |
| 17.....         | CH <sub>3</sub>                       | -CH <sub>2</sub> -S-CH <sub>2</sub> -S-CH <sub>2</sub> -                | 214                                  |

reducing agents, e.g., with the tin compounds described in Belgian Pat. Nos. 493,464 and 568,687; the imino-amino-methanesulfonic acid compounds described in Belgian Pat. No. 547,323 or with small quantities of noble metal compounds such as compounds of gold, platinum, palladium, iridium, ruthenium and rhodium. The emulsions may also be sensitized with polyalkylene oxide derivatives, e.g., with polyethylene oxide having a molecular weight of between 1,000 and 20,000, with condensation products of alkylene oxides and aliphatic alcohols, glycols and cyclic dehydration products of hexitols, with alkyl-substituted phenols, aliphatic carboxylic acids, aliphatic amines, aliphatic diamines and amides. These condensation products should have a molecular weight of at least 700, preferably more than 1,000. These sensitizers may, of course be combined in order to achieve particular effects, as is described in Belgian Pat. No. 537,278 and in British Pat. No. 727,982.

Instead of incorporating the antibronzing agents in the photographic copying material, they may be dissolved in one of the treatment baths. For example, they may be added to the developer, the fixing bath, or to an additional hardening bath or a bath which contains surface active compounds and which is used as the final treatment bath before the image containing material is dried at elevated temperature. The compounds according to the invention are generally dissolved in the bath as alkali metal salts in concentrations which may vary within very wide limits but generally lie between 10 and 100 mg. per liter, provided that the compounds are soluble in the fixing bath. Satisfactory results are obtained using, for example, 20 to 50 mg. per liter of the compounds in the developer bath or in the fixing bath. When the photographic copying material is passed through such a bath, the water permeable layers take up a certain amount of the antibronzing agent.

#### EXAMPLE 1

A silver chlorobromide gelatin emulsion (20 mols percent of AgBr) which is unwashed and which contains per liter 0.18 mol of silver halide, 2 ml. of a 1 percent alcoholic solution of 1-phenyl-5-mercaptopentazole, 20 ml. of a 10 percent aqueous saponin solution and 2 ml. of a 30 percent aqueous formalin solution is divided into eight portions. To each portion is added an antibronzing agent of the present invention. Details are given in the following table.

The emulsions are applied onto a baryta-coated paper support. The final dried layer contains 1.6 g. silver per square meter in the form of silver halide.

Comparison strips of the photographic material thus obtained is exposed in a sensitometer customarily employed in the art. The exposed samples are developed in a developer of the following composition (temperature 18° C., developing time 90 seconds):

1 g. of p-methylaminophenol  
3 g. of hydroquinone  
13 g. of anhydrous sodium sulfite  
26 g. of anhydrous sodium carbonate  
1 g. of potassium bromide dissolved in water and made up to 1,000 ml.

The developed material is fixed for 10 minutes in an aqueous solution of sodium thiosulfate and rinsed.

The moist material is dried on a high-gloss press heated to 130° C. Whereas the high-gloss drying causes a color change from brown to greenish brown to blue in the control sample (without addition), the brown image tones do not change if a compound according to the invention is present. The maximum density of the different materials is determined with a densitometer of an air-dried sample as compared with a material dried on a glazing press. The following results are obtained;

TABLE 2

| Compound from | Concentration | Maximum Density dried on |
|---------------|---------------|--------------------------|
|---------------|---------------|--------------------------|

| Table 1        | mg./kg. | Air dried | Glazing press |
|----------------|---------|-----------|---------------|
| Control sample | 0       | 2.30      | 1.72          |
| 1              | 166     | 2.28      | 2.33          |
| 3              | 238     | 2.31      | 2.43          |
| 5              | 166     | 2.28      | 2.40          |
| 6              | 182     | 2.33      | 2.41          |
| 7              | 254     | 2.32      | 2.42          |
| 8              | 211     | 2.35      | 2.39          |
| 9              | 185     | 2.31      | 2.30          |
| 10             | 14      | 2.29      | 2.33          |

#### EXAMPLE 2

15 A silver chloride emulsion which contains per liter 0.18 mol of silver chloride and the additives mentioned in Example 1 is divided into several portions. To each portion is added an antibronzing agent according to the invention as referred to in detail in the following Table 3. The compounds are added in the form of a solution in dimethylformamide as described in Example 1.

20 The emulsions are applied onto a baryta-coated paper support. The dried layer contains 1.35 g. silver in the form of silver chloride per square meter.

25 Further processing is accomplished as described in Example 1.

TABLE 3

| No. of compound from Table 1 | Concentration mg./kg. | Air dried | Maximum Density dried on glazing press |
|------------------------------|-----------------------|-----------|----------------------------------------|
| Control sample               | 0                     | 2.04      | 1.59                                   |
| 1                            | 166                   | 2.01      | 2.10                                   |
| 4                            | 168                   | 2.05      | 2.08                                   |
| 7                            | 254                   | 2.02      | 2.12                                   |
| 9                            | 185                   | 2.13      | 2.23                                   |
| 10                           | 153                   | 2.08      | 2.16                                   |
| 14                           | 150                   | 2.13      | 2.20                                   |
| Control sample               | 0                     | 1.94      | 1.58                                   |
| 2                            | 196                   | 1.94      | 2.00                                   |
| 3                            | 238                   | 1.96      | 2.01                                   |
| 5                            | 166                   | 1.96      | 2.11                                   |
| 6                            | 182                   | 1.99      | 2.10                                   |
| 8                            | 211                   | 1.97      | 2.08                                   |

#### EXAMPLE 3

50 Comparison strips of the photographic material of the control sample of Example 1 are processed as described in Example 1 but using developers that contain an antibronzing agent of the present invention in the amount indicated in the following table. The following results are obtained:

TABLE 4

| No. of compound from Table 1 | Concentration mg./l. | Air dried | Maximum Density dried on glazing press |
|------------------------------|----------------------|-----------|----------------------------------------|
| Control sample               | —                    | 2.24      | 1.78                                   |
| 1                            | 22                   | 2.24      | 2.27                                   |
| 2                            | 26                   | 2.24      | 2.31                                   |
| 3                            | 32                   | 2.24      | 2.36                                   |
| 4                            | 45                   | 2.24      | 2.41                                   |
| 5                            | 44                   | 2.24      | 2.42                                   |
| 6                            | 24                   | 2.24      | 2.34                                   |
| 7                            | 34                   | 2.24      | 2.37                                   |
| 8                            | 28                   | 2.24      | 2.33                                   |
| 9                            | 49                   | 2.24      | 2.37                                   |
| 10                           | 42                   | 2.24      | 2.37                                   |
| 14                           | 20                   | 2.24      | 2.15                                   |
| 15                           | 40                   | 2.24      | 2.31                                   |

75 Whereas the high-gloss drying produces a change from warm brown to a color varying from greenish brown to blue in the control sample, the warm brown image tone remains

unchanged when developed in a developer containing the antibronzing agent.

## EXAMPLE 4

The comparisons of Example 3 are repeated with the exception however that instead of adding antibronzing agents to the developer, such additions are made to the fixing bath, using a fixing bath of the following composition:

Fixing bath:

200 g. of sodium thiosulfate cryst.

20 g. of potassium metabisulphite dissolved in water and made up to 1,000 ml.

The fixing bath is divided into five equal portions before fixing. The compounds indicated in Table 5 below are added to these parts. The following results are obtained:

TABLE 5

| No. of compound from Table 1 | Concentration mg./l. | Maximum density Air dried | Maximum density dried on glazing press |
|------------------------------|----------------------|---------------------------|----------------------------------------|
| Control sample               | 0                    | 2.24                      | 1.78                                   |
| 1                            | 10                   | 2.24                      | 2.34                                   |
| 2                            | 20                   | 2.24                      | 2.43                                   |
| 9                            | 20                   | 2.24                      | 2.34                                   |
| 10                           | 20                   | 2.24                      | 2.41                                   |

Whereas high-gloss drying causes a color change from warm brown to greenish brown and then to blue in the control sample, the warm brown image tones do not change if fixing is performed in the presence of the antibronzing agent.

We claim:

1. In a process for the production of photographic images by exposing a supported silver halide emulsion layer, developing, fixing and hot drying, the improvement consisting of hot drying, the silver image in contact with an antibronzing amount of a compound of the following formula or its tautomeric 3-thione form:



wherein:

R is hydrogen, a saturated or olefinically unsaturated aliphatic group having up to six carbon atoms, a radical of the phenyl series or an amino group, and

X is an interrupted chain of two to 10 hydrocarbon groups, each interruption consisting of O, S, -NH-, or SO<sub>2</sub>.

2. A process as defined in claim 1, wherein the hydrocarbon groups are methylene groups, the number of such groups is not more than six, and the interruptions are oxygen, sulfur or sulfonyl groups.

3. A photographic element containing at least one light-sensitive silver halide emulsion layer and an antibronzing amount of a compound of the following formula or its tautomeric 3-thione form:



wherein:

10 R is hydrogen, a saturated or olefinically unsaturated aliphatic group having up to six carbon atoms, a radical of the phenyl series or an amino group, and  
X is an interrupted chain of two to 10 hydrocarbon groups, each interruption consisting of O, S, -NH-, or SO<sub>2</sub>.

15 4. A material of claim 3 wherein the hydrocarbon groups are methylene groups, the number of such groups is not more than six, and the interruptions are oxygen, sulfur or sulfonyl groups.

5. An aqueous photographic developer composition containing photographic developer and an antibronzing amount of a compound of the following formula or its tautomeric 3-thione form:



30 wherein:

R is hydrogen, a saturated or olefinically unsaturated aliphatic group having up to six carbon atoms, a radical of the phenyl series or an amino group, and

35 X is an interrupted chain of two to 10 hydrocarbon groups, each interruption consisting of O, S, -NH-, or SO<sub>2</sub>.

6. The developer composition of claim 5 wherein the hydrocarbon groups are methylene groups, the number of such groups is not over six, and the interruptions are oxygen, sulfur or sulfonyl groups.

40 7. A photographic fixing bath containing a silver halide solvent and an antibronzing amount of a compound of the following formula or its tautomeric 3-thione form:



45 wherein:

R is hydrogen, a saturated or olefinically unsaturated aliphatic group having up to six carbon atoms, a radical of the phenyl series or an amino group, and

55 X is an interrupted chain of two to 10 hydrocarbon groups, each interruption consisting of O, S, -NH-, or SO<sub>2</sub>.

8. The fixing bath of claim 7 wherein the hydrocarbon groups are methylene groups, the number of such groups is not more than six, and the interruptions are oxygen, sulfur or sulfonyl groups.

\* \* \* \* \*